

July 14, 1959

E. GREGORY

2,894,838

METHOD OF INTRODUCING HARD PHASES INTO METALLIC MATRICES

Filed Oct. 11, 1956



INVENTOR.  
ERIC GREGORY  
BY  
Kohsch and Kohsch  
ATTORNEYS

**METHOD OF INTRODUCING HARD PHASES  
INTO METALLIC MATRICES**

Eric Gregory, Hastings on Hudson, N.Y., assignor to Sintercast Corporation of America, Yonkers, N.Y., a corporation of New York

Application October 11, 1956, Serial No. 615,336

11 Claims. (Cl. 75—206)

The present invention relates to the production of a reinforced metal product and, more particularly, to a method of introducing a hard refractory oxide phase into a ductile metal matrix.

It is known that high temperature strength properties of certain ductile metals can be improved by the addition to the metals of a discrete hard phase, e.g.  $Al_2O_3$ , which increases the metal's resistance to deformation and enables it to sustain high stress at elevated temperatures for prolonged periods of time. Wrought aluminum products produced from fine aluminum powders exhibit such improved properties in comparison to aluminum products made by conventional casting. This is because aluminum powders are generally characterized by a surface oxide coating which remains in the final product as finely dispersed hard particles of  $Al_2O_3$ . These particles behave as slip inhibitors and it is largely this characteristic that stiffens the metal or alloy and raises its resistance to applied stress at elevated temperatures. The disperse hard phase acts as a deterrent to recrystallization and grain growth and thus inhibits or decreases the metal's tendency to weaken and soften at elevated temperatures.

There have been recent trends to employ this disperse phase hardening mechanism in stiffening heat resistant alloys, for example an alloy containing 80% nickel and 20% chromium. A given amount of hard phase, e.g. titanium carbide powder, is added to the foregoing type alloy in the powder form and the two mechanically mixed to obtain a uniform distribution of one in the other. The mixture is consolidated into a compact and then hot worked at an elevated temperature into a desired shape. The fine dispersion of the carbide stiffens the matrix of the alloy and confers additional resistance to deformation at high stresses at elevated temperatures. In order to obtain full benefit, the hard phase must be substantially insoluble in the matrix of the alloy, otherwise the alloy will lose its stiffness and weaken due to the solution of the hard phase in the matrix metal.

One of the disadvantages of the foregoing method of introducing hard phases into the matrix was the tendency for mechanically mixed materials to segregate. Because of this effect, it was not always consistently possible to maintain a perfect mixture. Even when the powders were blended under the best possible mixing conditions, there still remained the problem of segregation during storage, handling, processing, pressing, etc. If the powders were stored for any length of time and subjected inadvertently to extraneous vibration usually prevailing in buildings containing large presses, reciprocating vacuum pumps and other heavy industrial machinery and equipment, the powders would tend to segregate due to marked differences in densities and, unless the powders were remixed, the final product would not always exhibit the desired properties due to non-uniform distribution of the slip-inhibiting phase in the final product.

The present invention overcomes the foregoing difficulties by providing a method for insuring uniformity of the final product by enabling the production of a metal powder with a slip-inhibiting phase associated with it.

It is, therefore, an object of the present invention to provide a method of producing metal powder having a hard phase associated therewith prior to consolidating the powder into a solid shape, thereby insuring a uniform distribution of said hard phase throughout the final product.

Other objects will more clearly appear from the following description taken in conjunction with the accompanying drawing which compares deforming stresses at various temperatures of a product of the invention with a similar product produced by conventional methods.

The introduction of the hard phase is achieved by the liquid phase sintering of a refractory oxide-yielding composite metal powder with a solid ductile matrix metal powder of melting point above that of the metal in the composite powder, preferably above 750° C.

By refractory oxide-yielding powder is meant a metal powder having a propensity of forming a refractory oxide coating of high melting point, the metal underneath the coating having a melting point below that of said matrix metal powder, preferably below about 900° C. and more preferably within the range of about 600° C. to 900° C.

In carrying the invention into practice, a matrix metal powder is uniformly mixed and blended with sufficient refractory oxide-yielding composite metal powder characterized by a high melting point refractory oxide coating. The mixture is tamped into a confining mold, e.g. a steel tube, and then subjected to liquid phase sintering under reducing conditions at a temperature above the melting point of the metal in the composite powder but below the melting point of the matrix metal powder.

The molten refractory oxide-yielding metal breaks through its oxide coating and diffuses into the matrix metal, the refractory oxide shell which remains then becomes associated with the resulting alloyed powder. The liquid phase heating results in an agglomerated or fritted powder which is thereafter pulverized. The comminuted powder is then treated like any metal powder in forming a consolidated product. For example, the powder may be hot pressed into an ingot under neutral or reducing conditions and thereafter hot extruded at an elevated temperature into a desired shape. The resulting product will be characterized by a metal matrix having dispersed therethrough finely divided particles of refractory oxide and will exhibit improved resistance to creep above room temperature.

An example of a refractory oxide-yielding composite powder is aluminum. Finely divided aluminum powder when oxidized contains a refractory oxide surface coating and, depending on how the powder is produced, may contain oxygen (as  $Al_2O_3$ ) in amounts ranging from about 0.2 to 15% by weight of the powder. Atomized aluminum powder generally exhibits a low oxygen content (for example in the neighborhood of 0.5%) while very fine flake powder (e.g. minus 325 mesh, U.S. Standard screen size) can be produced having a higher oxygen content ranging as high as 15% by weight and even a little higher. This composite powder is ideal because first the melting point of the metal (about 660° C.) makes it desirable for liquid phase sintering with a solid matrix metal powder; second, the aluminum oxide is hard, stable and substantially insoluble in the matrix metal at elevated temperatures and, therefore, makes an excellent slip inhibitor; and, third, the oxide coating has a relatively high melting point (over 2000° C.).

Magnesium metal powder is another suitable material. Like aluminum, it forms a hard, stable oxide coating ( $MgO$ ) which has a high melting point (about 2500° C.)

compared to the much lower melting point of the metal itself (about 650° C.) and similarly is substantially insoluble in the matrix metal.

The rare earth metals such as cerium, lanthanum, neodymium, etc. could also be used, if desired, since they have melting points falling within the range of about 600° C. to 900° C. Cerium has a relatively low melting point in the neighborhood of 600° C., lanthanum in the neighborhood of about 825° C., and neodymium in the neighborhood of 840° C. Their oxides on the other hand melt at a much higher temperature of over 1600° C.

It will be apparent from the foregoing that the liquid phase sintering materials (i.e. Al, Mg, Ce, etc.) are all characterized by melting points below 950° C. while their respective oxides are hard and stable and have very high melting points in excess of 1600° C.

The matrix metals on the other hand have melting points above those of the refractory oxide-yielding metal, preferably above 900° C. Examples of matrix metals for the purposes of this invention are silver, gold, copper, platinum, palladium, nickel, cobalt, iron, and alloys based on one or more of these metals, etc. Such matrix metals may be selected broadly from the copper group, platinum group and iron group metals and their alloys. Other matrix metals may include tungsten, molybdenum, columbium etc.

The matrix metals are preferably defined broadly as those whose oxides have a negative free energy of formation at 25° C. below about 70,000 calories per gram atom of oxygen. In contrast the refractory oxide-yielding metal has a negative free energy of formation with oxygen of over 90,000 calories per gram atom of oxygen, and, generally, over 120,000. This difference of free energies between the oxide of the matrix metal and that of the refractory oxide-yielding metal is an important consideration as it enables the carrying out of certain preferred embodiments of the invention to be described later.

As illustrative of the invention, the following examples are given:

*Example I*

Fine flake copper powder (minus 200 mesh) and 8% by weight of very fine flake aluminum powder (minus 325 mesh) having an oxygen content of about 15% by weight of the aluminum powder are mechanically blended together and the mixture packed in a steel tube. The mixture is then heated in hydrogen to 900° C. and subjected to liquid phase sintering for one hour. The resulting fritted powder which has a yellowish bronze color is then pulverized, cold compacted, thereafter heated to 1000° C. in nitrogen, placed in a cold die and immediately hot pressed at 30 tons per square inch. The hot pressed billet is then machined, heated to 1000° C. and then hot extruded at a pressure of 50 tons per square inch and an extrusion ratio of 20 to 1 to form an extruded aluminum bronze alloy containing about 2.5% by weight of  $\text{Al}_2\text{O}_3$  as a slip inhibitor.

The drawing shows a comparison of properties of aluminum bronze produced in accordance with Example I (note curves (1) and (2)), with conventional cast or wrought aluminum bronze (3). The extruded material produced in accordance with this invention (1) was tested at various temperatures under stresses where appreciable deformation occurred. It will be noted that the alloy of the invention (1) can sustain higher loads before deforming appreciably at temperatures up to 500° C. than a conventional cast and wrought aluminum bronze alloy containing about 10% aluminum. Even when the invention alloy is soaked for a long period of 16 hours at 900° C., note curve (2), it still sustains higher loads before appreciably deforming.

*Example II*

The invention is also applicable to the production of age-hardenable magnesium-containing nickel alloys. In

producing a Ni-Mg alloy containing about 1% magnesium, powder nickel of minus 200 mesh is mixed with powder magnesium of minus 325 mesh containing about 10% by weight of oxygen as a surface layer of  $\text{MgO}$ . The mixed powders are tamped in a confining chamber and then heated in a reducing atmosphere and subjected to liquid phase sintering at a temperature of about 700° C. for about 1 hour (it is preferred that the temperature not exceed 700° C. or 750° C. in view of the relatively high vapor pressure of magnesium at high temperatures). The resulting fritted an alloyed powder is pulverized, cold compacted and thereafter heated to a temperature of about 800° C. in an inert atmosphere, placed in a cold die and immediately hot pressed at a pressure of 30 to 40 tons per square inch. The resulting billet is machined, sheathed airtight in an iron container, heated to 1000° C., and then hot extruded at a pressure of about 50 tons per square inch and an extrusion ratio of about 20 to 1 to form an extruded nickel alloy containing some magnesium in solid solution and some magnesium as a disperse hard phase of  $\text{MgO}$ . An addition of 1% magnesium having an oxygen content of about 10% will result in a nickel alloy containing  $\text{MgO}$  in the neighborhood of about 0.25% by weight.

*Example III*

Similarly, in forming a nickel-aluminum age-hardening alloy, e.g. an alloy containing about between 4 to 5% aluminum, somewhat the same procedure may be employed. In producing the alloy, about 5% of aluminum powder containing 15% oxygen is mechanically mixed with nickel powder (minus 325 mesh) and the mixture tamped into a mold. The mixture is then subjected to liquid phase sintering at a temperature of about 1000° C., whereby substantially all of the aluminum is alloyed with the nickel, the oxide shell remaining becoming associated with the alloy particles. A frit results which is pulverized to pass through 200 mesh. The pulverized mixture is then cold compacted and thereafter heated to a temperature of about 1000° C. in a reducing atmosphere and immediately placed in a cold die and hot compacted at about 30 to 40 tons per square inch, machined into an extrusion slug, sheathed airtight in an iron container and then finally hot extruded at about 75 tons per square inch at a temperature of about 1000 to 1050° C. and an extrusion ratio of 18 to 1 to form a nickel-aluminum alloy shape characterized by a fine dispersion of approximately 1.5%  $\text{Al}_2\text{O}_3$  by weight throughout.

Heat resistant alloys can likewise be similarly treated. For example, an alloy powder comprising 80% nickel and 20% chromium can be treated as above. Likewise heat resistant cobalt-base and iron-base alloy powders may be also treated.

Where a high oxide content is desired in the final product, for example an oxide content of about 5% or higher of  $\text{Al}_2\text{O}_3$ , this can be achieved by starting with a partially oxidized matrix metal powder which is reacted with aluminum or similar powder to produce the desired refractory oxide. In this respect it is important as indicated hereinbefore that the negative free energy of formation of the matrix metal oxide at about 25° C. be less than 70,000 calories per gram atom of oxygen, while that for the refractory oxide-yielding metal be at least greater than 90,000 and preferably greater than 120,000 calories per gram atom. Thus, nickel powder partially oxidized to an oxygen content of about 5% would be subjected to liquid phase sintering at about 1000° C. with flake aluminum powder containing about 15% oxygen. The nickel oxide ( $\text{NiO}$ ) having a negative free energy of formation of about 51,700 calories at about 25° C. will react with liquid aluminum and be reduced by it to nickel, the aluminum in turn being oxidized to  $\text{Al}_2\text{O}_3$ , since the negative free energy of formation of aluminum oxide at about 25° C. is of the order of 125,590 calories per gram atom. Thus, the  $\text{Al}_2\text{O}_3$  formed by reaction

augments the  $Al_2O_3$  already contained in the flake aluminum powder.

Assuming 92 parts of nickel powder containing 5% oxygen is reacted at 1000° C. with 8 parts aluminum flake powder containing 15% oxygen, and assuming the liquid phase reaction between aluminum and  $NiO$  goes to completion, the mixture will contain about 12.35% by weight of  $Al_2O_3$  the balance comprising about 87.4% nickel with a small amount of aluminum (about 0.25%) alloyed therewith. It is apparent from the foregoing that many variations can be resorted to in utilizing the advantages of the invention.

As illustrative of the type of ductile copper group, platinum group and iron group alloys that can be treated in accordance with the invention, the following is given:

Examples of copper group alloys are: 95% copper and 5% zinc; 90% copper and 10% zinc; 60% copper and 40% zinc; 71% copper, 28% zinc and 1% tin; 65% copper, 17% zinc and 18% nickel; 90% silver and 10% copper; up to 12% nickel and the balance silver; 70% gold and the balance palladium; 69% gold, 25% silver and 6% platinum, etc.

The copper group matrix metals and their alloys may be liquid phase sintered with such refractory oxide-yielding metals as aluminum at a temperature range above the melting point of the oxide-yielding metal, e.g. from about 700° C. to below the melting point of the matrix metal, usually within the range of 700° C. to 1000° C.

Examples of iron group alloys include: certain steels; 64% iron and 36% nickel; 31% nickel, 4 to 6% cobalt, and the balance iron; 54% iron and 46% nickel; 99% nickel and the balance cobalt; 68% nickel and 32% copper, etc. Heat resistant alloys based on the iron group metals can also be treated including stainless steels, and heat resistant nickel-base and cobalt-base alloys. The liquid phase sintering temperatures of the foregoing matrix metals with the refractory oxide-yielding metal may similarly range from 700° C. to below the melting point of the matrix metals, e.g. from 700° C. to 1200° C.

Examples of platinum group alloys are as follows: platinum-rhodium alloys containing up to 50% rhodium; platinum-iridium containing up to 30% iridium; platinum-nickel containing up to 6 or 10% nickel; platinum-palladium-ruthenium containing 77% to 10 platinum, 13% to 88% palladium, and 10% to 2% ruthenium; alloys of palladium-ruthenium containing up to 8% ruthenium; 60% palladium and 40% silver, etc. These alloys with refractory oxide-forming metal would be treated similarly as the copper group alloys.

When employing aluminum powder as the refractory oxide-yielding metal, it is preferred that the powder be non-leaving and have a particle size of less than 200 mesh and, preferably, less than 325 mesh. Other metal powders similar to aluminum should likewise be preferably maintained at minus 200 or 325 mesh.

The oxygen content of the refractory oxide-yielding powder may range broadly from about 0.2% to 15% by weight and may be liquid phase sintered with the matrix metal over the temperature range of 700 to 1200° C. In producing reinforced metal products, the composite powder produced in accordance with the invention is first consolidated before it is hot worked or extruded. It is preferred that the mixture be consolidated to an apparent density of at least about 65%, preferably as near as 90% as possible, before it is hot worked. While in general it would be preferred that the mixture be cold pressed, it will be appreciated that hot pressing can also be employed. In producing a compact of at least 65% apparent density by cold pressing, the pressure applied may range from 15 to 50 tons per square inch. When hot pressing is employed, the temperature will usually range from 650° C. to 1250° C. at pressures ranging up to about 40 tons per square inch, lower pressures being employed at higher temperature levels. Where high compacting pressure in conjunction with high temperature is

employed the billet is heated separately, placed in a cold die and immediately hot compacted. When hot pressing is conducted, it should be carried out under protective conditions, e.g. in a reducing atmosphere, an inert atmosphere or even at subatmospheric pressure.

Likewise when the compact is extruded, the conditions also should be protective to the materials forming the compact. Encasing the compact in an airtight, evacuated, welded container, for example a sheath of iron or nickel, is one method of protecting the materials in the compact from oxidation, etc. Depending on the situation, extrusion pressure may range from about 40 to 250 tons per square inch over a temperature range of about 800° C. to 1250° C. for extrusion ratio, ranging from about 14 to 1 and 20 to 1.

Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and appended claims.

I claim:

25. A method of introducing a hard slip inhibiting phase into a ductile matrix metal, an oxide of which has a negative free energy of formation at about 25° C. of below 70,000 calories per gram atom of oxygen which comprises providing a powder of said ductile matrix metal of melting point above 750° C. having mixed therewith a refractory oxide-yielding metal powder of melting point below that of the matrix metal and having a refractory oxide coating which is substantially stable at elevated temperatures and has a negative free energy of formation at about 25° C. of over 90,000 calories per gram atom of oxygen, subjecting said mixed powder to liquid phase sintering at an elevated temperature above the melting point of said refractory oxide-yielding metal and below the melting point of said matrix metal, whereby the refractory oxide-yielding metal melts, escapes from beneath its oxide shell and alloys with said matrix metal powder, the refractory oxide shell becoming associated with said alloy powder, consolidating said powder to a solid compact and hot forming said compact to a desired shape, 40 whereby said shape is characterized by a uniform dispersion throughout of particles of said hard refractory oxide.

2. A method of introducing a hard slip inhibiting phase into a ductile matrix metal an oxide of which has a negative free energy of formation at about 25° C. of below 70,000 calories per gram atom of oxygen which comprises providing a powder of said ductile matrix metal of melting point above 750° C. having mixed therewith up to about 10% by weight of at least one refractory oxide-yielding metal powder selected from the group consisting of aluminum, magnesium, cerium, lanthanum and neodymium of melting point below that of the matrix metal and having an oxygen content of about 0.2% to 15% in the form of a refractory oxide coating based on 55 said oxide-yielding metal which is substantially stable at elevated temperatures and has a negative free energy of formation at about 25° C. of over 90,000 calories per gram atom of oxygen, subjecting said mixed powder to liquid phase sintering at an elevated temperature above the melting point of said refractory oxide-yielding metal and below the melting point of said ductile matrix metal within the range of about 700 to 1200° C., whereby the refractory oxide-yielding metal melts, escapes from beneath its oxide shell and alloys with said matrix metal powder, the refractory oxide shell becoming associated with said alloy powder, comminuting said treated powder, consolidating said powder to a solid compact and hot forming said compact to a desired shape, whereby said shape is characterized by a uniform dispersion throughout 70 of fine particles of a hard refractory oxide.

3. A method of introducing a hard slip inhibiting phase into a ductile matrix metal of melting point above 750° C., an oxide of which has a negative free energy of formation at about 25° C. of below 70,000 calories per gram atom of oxygen, which comprises providing a powder of said matrix metal having mixed therewith up to about 10% by weight of finely divided aluminum powder characterized by an oxygen content of about 0.2% to 15% in the form of a refractory aluminum oxide coating whose negative free energy at about 25° C. is over 90,000 calories per gram atom of oxygen, subjecting said mixed powder to liquid phase sintering at an elevated temperature above the melting point of aluminum within the range of about 700 to 1200° C., whereby the aluminum melts, escapes from beneath its oxide coating and alloys with said matrix metal powder, the refractory aluminum oxide coating becoming associated with the particles of said alloy powder, comminuting said treated powder, consolidating said powder to a solid compact and hot forming said compact to a desired shape, whereby said shape is characterized by a uniform dispersion throughout of fine particles of said aluminum oxide.

4. A method of introducing a hard slip inhibiting phase into a ductile matrix metal an oxide of which has a negative free energy at about 25° C. or below 70,000 calories per gram atom of oxygen, which comprises providing a powder of said matrix metal of melting point above 750° C. with an oxidized surface and having mixed therewith refractory oxide-yielding metal powder of melting point below that of the matrix metal and having an oxygen content of about 0.2% to 15% by weight in the form of a refractory oxide coating based on said oxide-yielding metal which is substantially stable at elevated temperatures and has a negative free energy of formation at about 25° C. of over 90,000 calories per gram atom of oxygen, subjecting said mixed powder to liquid phase sintering at an elevated temperature above the melting point of said refractory oxide-yielding metal and below the melting point of said matrix metal, whereby the refractory oxide-yielding metal melts, escapes from beneath its oxide shell and reacts with the oxide coating on said matrix metal powder, reduces it with the consequent formation of more refractory oxide, the newly formed oxide together with the original refractory oxide becoming associated with said alloy powder, comminuting said treated powder, consolidating said powder to a solid compact and hot forming said compact to a desired shape, whereby said shape is characterized by a uniform dispersion throughout of fine particles of a hard refractory oxide.

5. A method of introducing a hard slip inhibiting phase into a ductile matrix metal of melting point above 750° C., an oxide of which has a negative free energy at about 25° C. of below 70,000 calories per gram atom of oxygen, which comprises providing a powder of said matrix metal with an oxidized surface and having mixed therewith at least one refractory oxide-yielding metal powder selected from the group consisting of aluminum, magnesium, cerium, lanthanum and neodymium of melting point below that of the matrix metal and having an oxygen content of about 0.2% to 15% by weight in the form of a refractory oxide coating based on said oxide-yielding metal which is substantially stable at elevated temperatures and has a negative free energy of formation at about 25° C. of over 90,000 calories per gram atom of oxygen, subjecting said powder to liquid phase sintering at an elevated temperature above the melting point of said refractory oxide-yielding metal and below the melting point of said matrix metal within the range of about 700° C. to 1200° C., whereby the refractory oxide-yielding metal melts, escapes from beneath its oxide shell, and reacts with the oxide coating on said matrix metal powder, reduces it with the consequent formation of more refractory oxide, the

newly formed oxide together with the original refractory oxide becoming associated with the particles of said alloy powder, comminuting said treated powder, consolidating said powder to a solid compact and hot forming said compact to a desired shape, whereby said shape is characterized by a uniform dispersion throughout of fine particles of a hard refractory oxide.

6. A method of introducing a hard slip inhibiting phase into a ductile matrix metal an oxide of which has a negative free energy of formation at about 25° C. of below about 70,000 calories per gram atom of oxygen, which comprises providing a powder of said matrix metal of melting point above 750° C. with an oxidized surface having mixed therewith finely divided aluminum powder characterized by an oxygen content of about 0.2% to 15% in the form of a refractory aluminum oxide coating whose negative free energy of formation at about 25° C. is over 90,000 calories per gram atom of oxygen, subjecting said mixed powder to liquid phase sintering at an elevated temperature above the melting point of aluminum and below the melting point of said matrix metal within the range of about 700° C. to 1200° C., whereby the aluminum escapes from beneath its oxide coating and reacts with the oxide coating on said matrix metal powder, reduces it with the consequent formation of new aluminum oxide, the newly formed oxide together with the original aluminum oxide becoming associated with the particles of said alloy powder, comminuting said treated powder, consolidating said powder to a solid compact and hot forming said compact to a desired shape, whereby said shape is characterized by a uniform dispersion throughout of fine particles of a hard refractory oxide.

7. A method of introducing a hard slip inhibiting phase into a ductile matrix metal powder, an oxide of which has a negative free energy of formation at about 25° C. of below 70,000 calories per gram atom of oxygen, which comprises providing a powder of said matrix metal of melting point above 750° C. having mixed therewith a refractory oxide-yielding metal powder of melting point below that of the matrix metal and having an oxygen content of about 0.2% to 15% in the form of a refractory oxide coating which is substantially stable at elevated temperatures and has a negative free energy of formation at about 25° C. of over 90,000 calories per gram atom of oxygen, subjecting said mixed powder to liquid phase sintering at an elevated temperature above the melting point of said refractory oxide-yielding metal and below the melting point of said matrix metal, whereby the refractory oxide-yielding metal melts, escapes from beneath its oxide shell, and alloys with said matrix metal powder with the refractory oxide coating thereafter becoming associated with said resulting alloy powder.

8. A method of introducing a hard slip inhibiting phase into a ductile matrix metal powder of melting point above 750° C., an oxide of which has a negative free energy of formation at about 25° C., of below 70,000 calories per gram atom of oxygen, which comprises providing a powder of said matrix metal having mixed therewith at least one refractory oxide-yielding metal powder selected from the group consisting of aluminum, magnesium, cerium, lanthanum and neodymium of melting point below that of the matrix metal and having an oxygen content of about 0.2% to 15% by weight in the form of a refractory oxide coating based on said oxide-yielding metal which is substantially stable at elevated temperatures and has a negative free energy of formation at about 25° C. of over 90,000 calories per gram atom of oxygen, subjecting said mixed powder to liquid phase sintering at an elevated temperature above the melting point of said refractory oxide-yielding metal and below the melting point of said matrix metal within the range of about 700° C. to 1200° C., whereby the refractory oxide-yielding metal melts, es-

capes from beneath its oxide shell and alloys with said matrix metal powder with the refractory oxide coating thereafter becoming associated with said resulting alloy powder and then comminuting said powder.

9. A method of introducing a hard slip inhibiting phase into a ductile matrix metal powder of melting point above 750° C., an oxide of which has a negative free energy of formation at about 25° C. of below 70,000 calories per gram atom of oxygen, which comprises providing a powder of said matrix metal having mixed therewith finely divided aluminum powder characterized by an oxygen content of about 0.2% to 15% in the form of a refractory aluminum oxide coating whose negative free energy of formation at about 25° C. is over 90,000 calories per gram atom of oxygen, subjecting said mixed powder to liquid phase sintering at an elevated temperature above the melting point of aluminum within the range of about 700° C. to 1200° C., whereby the aluminum melts, escapes from beneath its oxide coating, and alloys with said matrix metal powder with the refractory aluminum oxide coating thereafter becoming associated with said resulting alloy powder and then comminuting said powder.

10. A method of introducing a hard slip inhibiting phase into a ductile matrix metal powder an oxide of which has a negative free energy at about 25° C. of below 70,000 calories per gram atom of oxygen which comprises providing a powder of said matrix metal of melting point above 750° C. with an oxidized surface and having mixed therewith at least one refractory oxide-yielding metal powder selected from the group consisting of aluminum, magnesium, cerium, lanthanum and neodymium of melting point below that of the matrix metal and having an oxygen content of about 0.2% to 15% by weight in the form of a refractory oxide coating based on said oxide-yielding metal which is substantially stable at elevated temperatures and has a negative free energy of formation at about 25° C. of over 90,000 calories per gram atom of oxygen, subjecting said mixed powder to liquid phase sintering at an elevated temperature above the melting point of said refractory oxide-yielding metal and below the melting point of said matrix metal, whereby the refractory oxide-yielding metal melts,

5 escapes from beneath its oxide shell, and reacts with the oxide coating on said matrix metal powder, reduces it with the consequent formation of more refractory oxide, the newly formed oxide together with the original refractory oxide becoming associated with said resulting alloy powder.

10 11. A method of introducing a hard slip inhibiting phase into a ductile matrix metal powder an oxide of which has a negative free energy at about 25° C., of below 70,000 calories per gram atom of oxygen of melting point above 950° C. which comprises providing a powder of said matrix metal of melting point above 750° C. with an oxidized surface and having mixed therewith finely divided aluminum powder characterized by an 15 oxygen content of about 0.2% to 15% in the form of a refractory aluminum oxide coating whose negative free energy of formation at about 25° C. is over 90,000 calories per gram atom of oxygen, subjecting said mixed powder to liquid phase sintering at an elevated temperature above the melting point of said aluminum with- 20 in the range of about 700° C. to 1200° C., whereby the aluminum melts, escapes from beneath its oxide coating and reacts with the oxide coating on said matrix metal powder and reduces it with the consequent forma- 25 tion of more refractory oxide, the newly formed refractory oxide together with the original refractory aluminum oxide coating thereafter becoming associated with said resulting alloy powder, and then comminuting said powder.

30

References Cited in the file of this patent

UNITED STATES PATENTS

|           |              |               |
|-----------|--------------|---------------|
| 927,935   | Von Bolton   | July 13, 1909 |
| 2,100,537 | Conway       | Nov. 30, 1937 |
| 2,404,598 | Sachse       | July 23, 1946 |
| 2,657,128 | Stern et al. | Oct. 27, 1953 |
| 2,657,129 | Stern et al. | Oct. 27, 1953 |

FOREIGN PATENTS

|         |               |               |
|---------|---------------|---------------|
| 625,364 | Great Britain | June 27, 1949 |
| 160,526 | Australia     | July 17, 1952 |
| 730,931 | Great Britain | June 1, 1955  |